

Oct. 23, 1928.

1,688,381

H. M. DOWSETT ET AL

ELECTRICAL RESISTANCE

Filed June 16, 1925

Fig. 2



Fig. 1



Fig. 3



Fig. 4.

Inventor  
HARRY MELVILLE DOWSETT  
HERBERT BENJAMIN TILLEY

By their attorney  
Ina J. Adams

Patented Oct. 23, 1928.

1,688,381

# UNITED STATES PATENT OFFICE.

HARRY MELVILLE DOWSETT, OF COLCHESTER, AND HERBERT BENJAMIN TILLEY, OF CHELMSFORD, ENGLAND, ASSIGNORS TO THE RADIO CORPORATION OF AMERICA, OF NEW YORK, N. Y.

## ELECTRICAL RESISTANCE.

Application filed June 16, 1925, Serial No. 37,461, and in Great Britain June 17, 1924.

There is at present in general use a compact form of protected resistance unit which consists of a tube of unglazed porcelain wound with bare resistance wire which is sometimes 5 oxidized and coated with vitreous glaze. In the process of glazing, the tube is heated to a very high temperature so that no insulating or protective covering such as silk or 10 enamel can be used on the wire, and the metal employed for the wire must be such that it can be heated to this temperature without melting or changing its character. The number 15 of resistance alloys which can be employed for this purpose, is, therefore, strictly limited, particularly when wires of very small gauge are used, and it is found that alloys which have a very low or negligible temperature co-efficient cannot be employed. The porcelain tube and the finishing glaze 20 are both porous, so that the effective resistance, particularly of the high resistance units, varies with the moisture absorbed. The glaze as it is heated loses its insulating properties, and as in the process of manufacture the wire sometimes alters its position on the tube, and the oxide coating if employed is not a perfect insulator and is often patchy in character, the winding suffers from short 25 circuited turns.

30 The object of this invention is to obviate these disadvantages, and according to this invention a resistance is constructed as follows:—

(a) The tube is made of a refractory material which is impervious to moisture, such as glazed porcelain or glazed earthenware, or silica, or a suitable resistant glass.

(b) The wire is formed of any one of the well known resistance alloys, preferably one with a negligible temperature co-efficient.

The wire is enamel covered and then coated with a layer of silk, cotton or other absorbent material.

(c) The winding is impregnated with a suitable enamel and stoved for several hours at 150° C.

(d) The unit is then given a second coating of the same enamel and stoved for a longer period at a higher temperature.

(e) The second coating may be the finishing coat, or a third coating may be applied for this purpose, the tube being stoved finally at a temperature higher than the maximum working temperature, but such that the

enamel does not smoke or crack during the 55 stoving process, 250° C. being suitable.

A better understanding of the invention will be had from the specification when read in connection with the accompanying drawings in which:

Figure 1 shows in elevation a resistance unit made in accordance with this invention,

Figure 2 shows an end elevation of the unit shown in Figure 1,

Figure 3 shows at a larger scale a longitudinal section taken on the center line of Figure 1, while

Figure 4 shows in detail the successive steps taken in constructing a unit according to our invention.

Referring to these figures, 1 is a tube of refractory material which is impervious to moisture, and 2 an enamelled resistance wire having a negligible temperature co-efficient and covered with absorbent material 10 such as silk or cotton.

In order to form the end connections, only one of which is shown, a short length of pliable braided copper 3 is laid on the surface of the tube 1 as shown in Figs. 2 and 3, and lashed thereto by bare copper wire 4 for a distance of about  $\frac{1}{4}$  ", the said wire 4 having entwined with it a length of about 2 feet of resistance wire 2 which has been bared. The braided copper 3 is then turned back and soldered as shown at 5, the solder having a specially high melting point. The unit is then enamelled and stoved, as previously described, both layers of the enamel being indicated in Fig. 3 by the numeral 6. The enamel 6 is composed of 90 the layer of enamel 11 which is stoved at 150° and a second layer of enamel 12 which is then applied and stoved at a higher temperature.

7 is a clip, fitted round each end of the unit, and having a clamping screw 8 to which the braided copper 3 is secured as indicated in Figs. 1 and 2.

Such an end connection makes a good mechanical and electrical joint, and the flexible enamel coating 6 prevents any tendency of the solder to flow when the unit is under load.

It is found that the resistance of a unit made in this manner varies but very slightly, if at all, with increase of temperature; it can be run continuously at a normal temperature of 200° C. to 220° C.; there is no failure of insulation between turns; the unit is perfectly non-hygrosopic and is therefore suitable for

use under damp heat conditions such as are met with in the Tropics.

What we claim is:—

1. The process of manufacturing an electrical resistance unit which consists in winding an enamelled wire covered with absorbent material about a body of refractory material, impregnating the resistance unit so formed with enamel and stoving it, and subsequently applying a second coating of enamel to the resistance unit and stoving it at a temperature higher than the maximum working temperature.
2. The process of manufacturing an electrical resistance unit which consists in winding an enamelled wire covered with absorbent material about a body of refractory material, impregnating the resistance unit so formed with enamel and stoving it at a temperature below the normal working temperature, and subsequently applying a second coating of enamel to the resistance unit and stoving it at a temperature higher than the maximum working temperature.
3. The process of manufacturing an electrical resistance unit which consists in winding an enamelled wire covered with absorbent material about a body of refractory material, impregnating the resistance unit so formed with enamel and stoving it at a temperature

between 130° C. and 170° C. and subsequently applying a second coating of enamel to the resistance unit and stoving it at a temperature between 230° and 270° C.

4. The process of manufacturing an electrical resistance unit which consists in winding an enamelled wire covered with absorbent material about a body of refractory material, impregnating the resistance unit so formed with insulating material and stoving it and subsequently applying a second layer of insulating material to the resistance unit and stoving it at a temperature higher than the maximum working temperature of the unit.

5. The process of manufacturing an electrical resistance unit which consists in winding an enamelled wire covered with absorbent material about a body of refractory material, impregnating the resistance so formed with a plurality of layers of insulating material stoving one of said layers at a temperature below the normal working temperature and another of said layers at a higher temperature than the maximum working temperature.

In testimony that we claim the foregoing as our invention we have signed our names this fourth day of June, 1925.

HARRY MELVILLE DOWSETT.  
HERBERT BENJAMIN TILLEY.